

Feb. 4, 1958

J. F. JORDAN

2,822,258

## METHOD OF PRODUCING METALS FROM THEIR CHLORIDES

Filed Feb. 7, 1955

3 Sheets-Sheet 1



**FIG. I**

**INVENTOR: -**

James Fernando Forder

Feb. 4, 1958

J. F. JORDAN

2,822,258

METHOD OF PRODUCING METALS FROM THEIR CHLORIDES

Filed Feb. 7, 1955

3 Sheets-Sheet 2



INVENTOR: -

James Fernando Jordan

Feb. 4, 1958

J. F. JORDAN

2,822,258

METHOD OF PRODUCING METALS FROM THEIR CHLORIDES

Filed Feb. 7, 1955

3 Sheets-Sheet 3



INVENTOR:

*JAMES FERNANDO JORDAN*

1

2,822,258

## METHOD OF PRODUCING METALS FROM THEIR CHLORIDES

James Fernando Jordan, Huntington Park, Calif., assignor of one-third to the estate of James Jordan, deceased

Application February 7, 1955, Serial No. 486,591

12 Claims. (Cl. 75—43)

My invention relates to metallurgy.

This is a continuation-in-part of my copending applications: Serial No. 316,764 of October 24, 1952, Serial No. 316,765 of October 24, 1952, and Serial No. 331,301 of January 14, 1953; all abandoned.

Certain of the non-metallic constituents of steel have a damaging effect on the characteristics of steel. Of these, sulphur, oxygen, nitrogen and hydrogen are the worst offenders. All of these elements, or compounds of these elements, are soluble, at least to a minor extent, in steel at room temperature, and this soluble portion markedly influences the properties of the grains which, to a large extent, comprise the steel's structure. Such soluble impurities affect the magnetic and electrical properties of the metal and are thought to cause the yield point and determine the value of yield stress.

The insoluble portion of such impurities is formed as the molten steel is cooled to room temperature. During the cooling process, hydrogen tends to move into austenite remaining after the critical range has been passed, thereby forming islands of hydrogen concentration which, when the austenite transforms to martensite at a lower temperature, comes out of solution to form concentrated stresses, due to entrapment. When the structure as a whole is put under stress, such as when a test bar is pulled, these points of concentrated hydrogen stress act to control the behavior of the metal by acting to interfere with the normal operation of the slip and cleavage planes of the metal's grains.

Sulphur, oxygen and nitrogen precipitate from solution as sulphides, oxides, silicates and nitrides. That portion of these non-metallies whose precipitation occurs during the crystallizing phases of the cooling process are ejected by the crystallizing process to form on the grain boundaries of the metal's structure. It has been estimated that as little as 2 p. p. m. of such precipitated compounds can completely coat all of the grain boundaries of steel having grain sizes from ASTM Nos. 1 thru 10. In view of the fact that the grain boundaries form the continuous phase of the steel's structure, it may be seen that such grain boundary precipitation can exert an overriding influence on the properties of the steel; for these precipitated compounds, while apparently quite strong, are not ductile. Two outstanding examples of this are the brittle "rock candy" structure associated with the precipitation of aluminum nitride on the grain boundaries and the brittle eutectic sulphide fracture associated with the precipitation of aluminum sulphide on the grain boundaries.

Not all non-metallies act in these manners, carbon being an outstanding example. Due, in part, to its diffusibility in iron, carbon can be caused to avoid precipitating on the grain boundaries in the form of a brittle carbide, thus restricting its action to the discontinuous grains defined by the continuous grain boundary structure. Under such circumstances, the precipitated carbides act within the grains to interfere with the normal slip and cleavage planes to the end that each grain ex-

2

hibits a resistance to flow in all directions, even to the extent that the habit and degree of such precipitated carbides may be varied by heat treatment to vary the resistance to flow of the metal, as evidenced, for example, by the phenomenon known as: hardness.

When the prevalence of intercrystalline fracture is completely removed by forming the steel's structure under conditions that cause the grain boundaries to be clean, the ductility of the steel at high hardness levels is remarkably improved, almost to the extent that it may be characterized as a completely different metal.

It is well known that, the lower the sulphur, oxygen, nitrogen and hydrogen content of the steel, the better is the steel's ductility. As a result, conventional steel-making processes aim at carrying these impurities as low as possible. This objective is achieved in conventional processes by employing various techniques for removing such impurities from the metal. Thus, conventional practices involve allowing the impurities to get into the molten metal and then, by various techniques, lowering them to a level that permits the steel to meet conventional physical standards.

Unfortunately, even the best of these refining techniques are incapable of entirely eliminating these unwanted non-metallic impurities. Even the vacuum melting/vacuum casting technique can only lower these impurities, never eliminate them. As a consequence, steel today exhibits properties controlled, in large measure, by the degree and type of grain boundary contamination, rather than by the intrinsic properties of the grain.

I have found a method of producing steel that is essentially free of such non-metallic grain boundary films. Steel produced by my process exhibits the properties of the grain rather than the properties of the non-metallic film deposited on the grain boundaries.

In addition to iron and its alloys, such as steel, certain other metals and alloys thereof are adversely influenced by such non-metallic impurities; specifically, chromium, vanadium, nickel, cobalt, titanium and zirconium. These 40 metals and their alloys may be produced by my process with striking improvement in their physical properties.

My process involves the procedure wherein the occurrence of these grain boundary films is prevented by preventing these non-metallic elements from getting into the molten metal in the first place.

It is well known that the ores of these metals can be converted to chlorides that are essentially free from these non-metallic elements. And it is well known that such pure chlorides can be reduced to yield the desired product metal by means of the reducing agents: magnesium, sodium, potassium, lithium and calcium. When these chlorides are reduced in an environment that is completely free from hydrogen, oxygen and nitrogen by one of these reducing agents that is also free from these 55 non-metallic elements, the product metal content of the reaction mass from the chloride reduction process has the desired purity. The trouble is that the product metal content of the reaction mass is not in a consolidated form, but must be processed by a series of steps which always 60 introduce oxygen and nitrogen into the final metal form, and usually hydrogen as well.

Recognizing this, a recent investigator, Maddex, proposed that the reaction mass consisting of particles of the product metal entrained in a stream of molten magnesium chloride be flowed directly into contact with the surface of a pool of molten titanium, so that the heat of said pool will melt and accumulate said particles and so that the molten magnesium chloride will be vaporized. This proposal involves pouring molten magnesium chloride (B. P. 1691° K.) on the surface of a pool of molten titanium (M. P. 2000° K.). This is not 70 commercially feasible, for the same reason that it is not

feasible or safe to pour water (B. P. 373° K.) on the surface of a pool of molten lead (M. P. 601° K.).

Reactions of the subject type are strongly exothermic. A number of investigators, including the present inventor, have suggested that advantage be taken of this reaction heat to the end that the products issuing from the reaction zone are at a temperature that lies above the melting point of the product metal, thereby causing the byproduct reducing agent chloride to be in gas phase so that it will in no way interfere with the deposition of the molten product metal particles which are caused to impinge into contact with the surface of the pool of molten product metal in the collecting phase of the process.

The main difficulty with this proposal is that the heat released by these reactions is not sufficient to raise the reaction products to the desired temperature without preheating the reactants sufficiently to lift them over their respective boiling points, with the result that, in order to gain the desired temperature level, the reactants must be introduced into the reaction zone in gas phase. The resulting vapor phase reaction yields product metal particles whose state of subdivision is so fine that it resembles smoke. While product metal particles can be successfully deposited by such a hot reaction product stream, it is desirable that the efficiency of the deposition be substantially increased, so as to increase the process yield. The efficiency of the deposition is increased as the fineness of the product metal particles is decreased, the best results being obtained when the product metal particles are produced in a reaction in which the reaction zone is maintained at a temperature that lies between the boiling points of the reactants; that is, at a temperature at which one of the reactants, such as ferric chloride, is a gas and the other reactant, such as magnesium, is a liquid.

Figure 1 shows my process wherein product metal particles dispersed within a stream of molten reducing agent chloride, produced in a separate process, are caused to flow into my separate, but contiguous, temperature build up and depositing zones.

Figure 2 shows my process wherein said stream of molten reducing agent chloride containing product metal particles is formed in a reaction zone that is separate, but contiguous, to said temperature build up zone.

Figure 3 shows my process wherein said reaction zone is divided into two separate, but contiguous, reaction zones.

Various methods are available for forming the stream of molten reducing agent chloride containing product metal particles employed in the process of Figure 1. My U. S. Patent No. 2,647,826 discloses one such method. Another such method was disclosed by Maddex and Eastwood in the Journal of Metals, vol. 188, No. 4, April 1950. Other methods will occur to those skilled in the art.

Figure 1 shows my temperature build up 33 and depositing zones 35 cooperating to separate and accumulate in consolidated form the product metal particles (iron) entrained in a stream of molten reducing agent chloride (magnesium chloride), said iron bearing stream of magnesium chloride being a product of a separate reaction zone (not shown) in which iron chloride is reacted with magnesium. The products of a reaction between one of the subject metal chlorides and one of the subject reducing agents will hereinafter be referred to as: the reaction products. In Figure 1, a stream of molten magnesium chloride containing iron particles is caused to flow into the top of an elongated chamber to form a free falling stream of reaction products 31 within said chamber, said free falling stream being either continuous or a stream of discrete drops of molten magnesium chloride containing iron particles. As said stream of reaction products falls thru said chamber it flows into my temperature build up zone wherein the falling stream is mixed

with a concurrently flowing stream of a heating gas 30 formed in a refractory reaction vessel 29 between magnesium 27 and chlorine 28:



Reaction 1 releases a much larger amount of heat than is necessary to maintain the product chloride in the gas state; the heat content of the product chloride of reaction 1 in excess of that required to maintain said product chloride in the gas state is heat available for the temperature build up phase of my process.

In the temperature build up zone of my process, the available heat content of said heating gas is employed to evaporate the molten magnesium chloride content of

15 the falling stream of reaction products to form a heated stream 34 consisting of iron particles entrained in a stream of magnesium chloride gas, said heated stream being at a temperature that lies above the boiling point of magnesium chloride under the conditions obtained 20 between the temperature build up and depositing zones of my process. The amount of heating gas required to achieve this end will depend upon the design of the vessel that forms said chamber—to be discussed later; the amount and temperature of the reaction products 25 being flowed into the temperature build up zone; and the available heat content of the heating gas. In any case, sufficient of said heating gas is mixed with the falling reaction products within the temperature build up zone to form therein said heated stream.

30 The heated stream leaving the temperature build up zone is immediately flowed into a contiguous depositing zone 35 wherein said heated stream is flowed downward into contact with a surface 36 of a mass of the product metal, said surface being maintained at a temperature 35 that lies above the boiling point of the magnesium chloride content of said stream by means of the heat content of the heated stream impinging into contact with said surface. As said heated stream is impinged into contact with said surface, iron particles in said heated stream are 40 thrown into contact with and deposit on said surface.

The heated stream, containing such iron particles as are not deposited on said surface, is flowed from said surface out of said depositing chamber by means of an outlet positioned at a location that is sufficiently remote 45 from said surface to prevent the outflow of the byproduct gas stream from the deposition process from interfering substantially with the downward flow of the heated stream as said heated stream moves from the temperature build up zone to the depositing surface. In view of the large 50 volume of gas that must be handled in my process, per unit weight of deposited metal obtained, the outlet (not shown) in the wall of the depositing chamber must be large enough or numerous enough to prevent an excessively high gas back pressure from building up within 55 my process vessel, not only because of the complications that such high back pressure creates in the design of the vessel, but also because of the influence of high pressure on the boiling points of the components of the heated stream, etc.

60 The byproduct gas stream leaving the depositing chamber outlet may be recovered or disposed of in any convenient manner. The preferred method of handling the byproduct gas stream is to introduce an excess of chlorine into it after it leaves or just before it leaves the depositing chamber and then separating the resulting mixture of ferric chloride and magnesium chloride by fractional condensation procedures; the ferric chloride being re-cycled back into reaction 2, below, the magnesium 65 chloride being re-cycled back into the electrolytic process wherein the magnesium and chlorine are produced. Other methods of handling/utilizing the components of the byproduct gas stream will occur to those skilled in the art.

75 The reaction product stream being introduced into the

temperature build up zone or my process was presumably formed in a reaction where



Reaction 2 may be carried out with a moderate excess—say, 5%—of either ferric chloride or magnesium. When the reaction is carried out with a stoichiometric excess of ferric chloride, the reaction product stream will contain ferrous chloride; when it is carried out with a stoichiometric excess of magnesium, the reaction product stream will contain magnesium. Reaction 1 may be carried out with a stoichiometric excess of either chlorine or magnesium, such excess appearing in the heating stream. The heated stream emerging from my temperature build up zone will reflect equilibrium between all reactants, including such reactant excesses. For example, if reaction 1 is carried with a stoichiometric excess of chlorine, and the reaction product stream contains no magnesium, or not enough magnesium to combine with all of such excess chlorine, the uncombined chlorine will oxidize the finer iron particles to iron chloride in the temperature build up zone. Other effects arising from the use of stoichiometric excesses of reactants in reactions 1 and 2 will occur to those skilled in the art.

As the iron particles are deposited on the surface of the collecting mass within my depositing chamber, said surface will tend to rise towards the temperature build up zone, an action that is prevented, in my preferred embodiment, by withdrawing the mass forming said depositing surface downward at the same rate that said surface is being built up by the depositing iron particles, thus maintaining the distance between the temperature build up zone and the depositing surface at a substantially constant value.

The depositing surface of my process may be either solid iron or molten iron, the latter being my preferred embodiment, as shown in Figure 1. When the depositing surface is the surface 36 of a pool 8 of molten iron, said pool is retained in a water-jacketed mold 12 of the continuous type within which the molten depositing surface is maintained and supported by iron 37 that has been solidified at interface 9 by the cooling action of said mold, the position of said surface with respect to the temperature build up zone being controlled by withdrawing the supporting mass of solidified iron out of the bottom of said mold at the same rate that said surface tends to rise in said mold as the result of the depositing process taking place on said surface. The withdrawal of the solidified iron out of the bottom of said mold may be controlled in any convenient manner, such as by one or more sets of pinch rolls, such as is conventional in molds of this type.

The process of Figure 1 may be employed to separate and consolidate the product metal particles produced in reactions involving a chloride of a metal selected from the group consisting of, in addition to iron, chromium, vanadium, nickel, cobalt, titanium and zirconium that is reduced to yield the subject product metal by means of a reducing agent selected from the group consisting of magnesium, sodium, potassium, lithium and calcium. And said process may be employed to produce a consolidated metal product consisting of an alloy in which one of the listed product metals is the base or predominating metal. The product metal producing reaction involved in forming the reaction product stream of Figure 1 is not a part of the invention constituting the disclosure of Figure 1, however, in order to be employable in the process of Figure 1, said product metal producing reaction must yield or by means of the addition of a melting step must be capable of yielding the reaction product stream of Figure 1, said reaction product stream consisting of the molten reducing agent chloride from said reaction, together with the product metal particles dispersed therein, it being understood that the reaction product stream from such metal producing reactions may also contain the reducing agent or a chloride of the product metal,

depending upon the manner in which the metal producing reaction is carried out.

While Figure 1 shows my process being carried out in a completely water-jacketed vessel 32 containing circulating water 7, in order to assure the complete absence of contaminating refractories, air and hydrogen from the environment of my process, good results may be obtained without going to this extreme in certain cases wherein a refractory suitably resistant to the product metal is available. In the production of iron, for example, the temperature build up zone may be formed of a vessel lined with magnesia. It is important, however, in such a case, that reaction 1 be carried out with an excess of magnesium, for chlorine is reactive with magnesia.

The ability of the process of reaction 1 to achieve substantially complete product metal purity with respect to the aforementioned non-metallic impurities depends, in large measure, on the purity of the reactants employed in reaction 1 and the purity of the reaction product stream with respect to these non-metallics. Thus, the ferric chloride and magnesium being reacted to yield the reaction product stream must be free from these non-metallics, as must the chlorine and magnesium employed in reaction 1. In this connection, all commercially-available magnesium seems to contain magnesium oxide, magnesium nitride and hydrogen. The magnesium reagent should preferably be freed of these impurities by first subjecting it to a vacuum treatment at a temperature in the vicinity of its melting point to eliminate hydrogen, and then distilling the magnesium away from the oxide and nitride in a vacuum at as low a temperature as possible. It is a noteworthy feature of my process that the high-temperature heat required for this distillation is available as a by-product of my process; the heat content of the by-product gas stream 6 emerging from the product metal depositing zone being available for this purpose. The distilled reducing agent, whether it be magnesium, sodium, potassium, lithium or calcium, should be kept out of contact with air and vaporous water until it is passed into reactions 1 and/or 2, preferably with a blanket of helium or argon.

As mentioned previously, the reaction product stream may be caused to contain magnesium. If desired, the magnesium content of such a reaction product stream may be employed to heat said stream by reacting said magnesium with chlorine in the temperature build up zone. There are a number of ways in which this may be done. One such way involves forming a heating stream by employing a stoichiometric excess of chlorine, the excess chlorine reacting with the magnesium content of the reaction product stream when said stream is mixed with said heating stream. Another method involves the introduction of chlorine instead of the heating stream into the temperature build up zone, so that the reaction between said introduced chlorine and the magnesium content of the reaction product stream within the temperature build up zone will gain the desired gain in temperature. It is therefore apparent that reaction 1 may be caused to yield the desired temperature build up by a reaction that takes place within or outside of said zone, or by means of a combination of these reaction sites.

The product metal producing reaction by which the reaction product stream of Figure 1 is obtained may be carried out in any manner that will yield a product metal particle size capable of rapidly settling out of a moving stream of gas, and this particle size requirement, in turn, is predicated, in part, on the specific gravity of the product metal being produced. In other words, a larger particle size is required with titanium than with iron.

I prefer to carry out the metal producing reaction within the same vessel as that in which I am carrying out the temperature build up and depositing phases of my process. Figure 2 shows such an embodiment. The process of Figure 2 has the merit of being a synchronous process in which the metal producing zone, the tempera-

ture build up zone and the depositing zone are arranged in a straight-line flow wherein each step, while being substantially separate from the adjoining step(s), is contiguous thereto, so that the production rate of each step conforms to the production rate of the step(s) adjoining it.

As shown in Figure 2, this preferred embodiment involves positioning a water-jacketed conduit 44 containing cooling water 17 that is suitable for conducting a flowing stream of fluids in a vertical position directly over a horizontally-positioned product metal surface 43, said conduit being arranged and adapted to conduct said stream towards, and so into contact with, said surface, and then employing said conduit as a reaction chamber within which said three zones are arranged in chronological order.

In the uppermost of these three zones, the reaction product stream 31 is formed by reacting therein the reactants of reaction 2; that is, magnesium 27 and ferric chloride gas 40. This, the product metal producing zone, will hereinafter be called the primary reaction zone 49. Within the primary reaction zone, ferric chloride gas and molten magnesium are reacted to form the reaction product stream that immediately flows into the temperature build up zone 33, said stream consisting of one or more substantially continuous streams of molten magnesium chloride containing the iron in dispersed phase, or said stream may consist of a stream of discrete particles of molten magnesium chloride containing said dispersed iron phase.

In the temperature build up zone, the reaction product stream of Figure 2 is shown being heated to the desired temperature by means of a heating stream(s) 30 obtained according to reaction 1 in a separate zone (not shown) said streams 30 being introduced into the vessel via refractory conduits 45. If the reaction product stream emerging from the primary reaction zone of Figure 2 is caused to contain magnesium by employing therein a stoichiometric excess of magnesium, said excess may be oxidized in the temperature build up zone, if desired, by causing the heating stream to contain chlorine—for example, by employing a stoichiometric excess of chlorine in reaction 1. The basic function of the temperature build up zone is to lift the reaction product stream from a temperature that lies below the boiling point of magnesium chloride, preferably from a temperature that lies below the boiling point of magnesium, to a temperature that lies above the boiling point of magnesium chloride, preferably above the melting point of iron.

The heated stream flowing out of the temperature build up zone 33 is immediately flowed into the depositing zone wherein iron particles within said heated stream are caused to separate from the gaseous components of the heated stream by impinging said heated stream into contact with the surface 43 of a mass of the product metal (iron), the temperature of said surface being maintained at a level that lies above the boiling point of magnesium chloride, preferably above the melting point of iron, by means of the heat content of said heated stream. The heated stream, having given up particles of iron to said surface, now flows out of the depositing chamber as the byproduct gas 16 by means of outlet(s) positions in and penetrating thru the wall of the chamber that contains said product metal depositing zone, the byproduct gas outflow being arranged so that the gas outflow does not interfere substantially with the flow of the heated stream towards the depositing surface.

The depositing surface is shown, in Figure 2, contained in and supported by a water-jacketed mold of conventional continuous type, said mold acting to cause the depositing surface to seal and close the bottom of the depositing chamber. As in the case of the process of Figure 1, as the iron particles deposit on the depositing surface, the solidified iron shape 41 is withdrawn

7 downwards in order to maintain the depositing surface that it supports at a substantially constant level within the water-cooled mold, said shape 41 being formed at interface 15 from pool 42.

Reaction 2 must be carried out within the primary reaction zone in manners which cause said zone to be maintained at a temperature that lies below the boiling point of magnesium chloride (1691° K.), preferably at a temperature that lies between above the melting point of magnesium chloride (987° K.) and below the boiling point of magnesium (1399° K.). The lower the operating temperature of the primary reaction zone is maintained within this range, the larger will be the size of the product metal particles produced therein, and the more efficient will be the product metal collection process taking place within the depositing zone.

The operating temperature of the primary reaction zone may be controlled by controlling the amount of reactants being reacted therein within an interval of time; by controlling the cooling effect of the wall of the vessel containing said zone; by feeding an agent that is inert towards the reactants and resultants, such as helium or argon, into said zone; by controlling the temperature of the reactants being fed into said zone; by controlling the size of a stoichiometric excess of magnesium being fed into said zone; or by controlling a combination of these controlling expedients.

When the primary reaction zone is being operated with the view of maintaining the maximum production rate—the usual case, or when one of the more active reducing agents, such as lithium, is being employed, ordinary methods of holding down the operating temperature of the primary reaction zone will not suffice. Under such circumstances, I hold the operating temperature of the primary reaction zone within the desired limits by increasing the size of the stoichiometric excess of magnesium being fed into said zone. For example, if the operating temperature of the primary reaction zone is being held at, say, 1380° K., and for one reason or another the temperature of said zone begins to mount towards the boiling point of magnesium (1399° K.), I act to offset the rising temperature by increasing the amount of molten magnesium being fed into said zone until said temperature has fallen back to said 1380° K. The extra, heat quenching magnesium added in this manner may be oxidized in the temperature build up zone by feeding chlorine into said zone, or said extra magnesium may be recovered from the by-product gas after it leaves the depositing zone. The use of molten magnesium in this manner is particularly effective when it is being employed to hold the primary reaction zone operating temperature below the boiling point of magnesium, due to the temperature rise barrier: the heat of vaporization of magnesium. When, on the other hand, the temperature of the primary reaction zone begins to fall below the desired operating temperature, I act to lift the temperature to the desired level by cutting back on the amount of stoichiometric excess of magnesium being fed thereto.

The metal producing zones of processes such as this are not restricted to the reduction of ferric chloride, of course, there being certain advantages in employing therein the reaction wherein:



The preferred primary reaction zone operating temperature for reaction 3 is between above the boiling point of ferrous chloride (1299° K.) and below the boiling point point of magnesium (1399° K.), however, any temperature up to below the boiling point of magnesium chloride may be employed. The ferrous chloride of reaction 3 may be produced in any convenient manner, such as:



or



Reaction 5, of course, yields a mixture of chlorides; however, such a mixture may be reduced according to reaction 3 to yield the reaction product stream of my process. Success with reaction 5 requires certain precautions. If the chloride mixture product of reaction 5 is to be kept substantially free of iron, a substantial excess of ferric chloride over the indicated stoichiometric requirements must be fed into the reaction area where reaction 5 is being conducted. When, in the presence of a stoichiometric excess of ferric chloride, an iron phase separates, due to total excesses of magnesium, said excess ferric chloride at once oxidizes the separated iron phase according to reaction 4. In carrying out the two-step reduction of iron chloride according to reactions 5 and then 3, I prefer the procedure pictured in Figure 3; for, in Figure 3, the addition of the extra reduction step does not interfere with the highly desirable synchronous procedure as outlined in Figure 2.

In Figure 3, magnesium 27 is reacted with a stoichiometric excess of ferric chloride 40 in the uppermost dichloride zone 50, and the stream of ferrous chloride and magnesium chloride containing the excess ferric chloride then moves into the primary reaction zone 47 wherein a stoichiometric excess of magnesium gas 27 is reacted with said dichloride to yield the reaction product stream 30 of my process. The reaction product stream thereupon enters the temperature build up and depositing zones 33 and 35 of my process. Figure 3 shows a species of my temperature build up procedures not shown in Figures 1 and 2. In Figure 3, sufficient excess magnesium is fed into the primary reaction zone to provide the temperature build up zone with the magnesium required by reaction 1, reaction 1 being carried out within the temperature build up zone itself by mixing chlorine 28 with the reaction product stream as it enters said zone.

#### *The byproduct chloride*

As was mentioned previously, the reducing agent chloride of the reaction product stream and the reducing agent chloride of reaction 1 leave the depositing zone in the form of gas, that is, gas 6, 16 and 24, respectively. Depending upon how reaction 1 is carried out, this byproduct chloride gas will contain, in addition to the chloride of the reducing agent, uncollected particles of the product metal and unreacted reducing agent in gas phase, or said byproduct will contain a chloride of the product metal—in the latter case said gas may also contain uncollected product metal particles. Three things are of interest concerning this byproduct gas: (1) its heat content, (2) the reducing agent chloride that it contains, and (3) its metal content. Efficiency would suggest that the heat content of the byproduct chloride gas be utilized in the overall process for some useful purpose, such as the distillation of the reducing agent in order to purify it. In view of the fact that the reducing agent and chlorine are employed in large quantities in my process, it would seem apparent that the reducing agent chloride byproduct must be treated electrolytically to recover the reducing agent and chlorine for recycling back into reactions 1 and 2. In order that this may be carried out, the byproduct chloride gas must be freed from its metal content. In my preferred embodiment, the heat of vaporization of the reducing agent chloride gas is utilized for distilling the reducing agent, the distilling process being caused to yield, in addition to the purified reducing agent, molten reducing agent chloride containing impurities, such as particles of the product metal and/or a chloride of the product metal. If the condensed reducing agent chloride is at a temperature that lies above the boiling point of the reducing agent, any reducing agent present in the byproduct chloride gas may be separated from the molten reducing agent chloride by merely drawing the reducing agent gas off. With the reducing agent chloride collected in the form of a molten pool, I purify it and recover the product metal from it by passing chlorine

into and thru the molten pool, said chlorine acting to oxidize the product metal particles and such lower product metal chloride(s) as may be present to the higher, volatile product metal chloride, such as ferric chloride, titanium tetrachloride, zirconium tetrachloride, etc. The vaporous product metal chlorides produced by this chlorine oxidation are withdrawn from the molten pool to be condensed separate from said molten pool, and so recovered for recycling back into the product metal producing reaction; the purified reducing agent chloride of said molten pool being passed to the electrolytic process wherein the reducing agent and chlorine are produced. The product metal content of the byproduct chloride gas emerging from the depositing zone may also be recovered from said gas by merely feeding enough chlorine into the byproduct chloride gas after said gas emerges from the depositing zone to oxidize the product metal particles to the highest state of oxidation obtainable at the temperatures involved; that is, in the case of iron, ferric chloride, or in the case of titanium, titanium tetrachloride. With the product metal oxidized, the product metal chloride produced thereby is separated from the reducing agent chloride by fractional condensation.

#### *Alloys*

While I have employed the reaction wherein an iron chloride is reduced with magnesium to illustrate how my process functions, as mentioned previously, other metals may be produced by my process and other reducing agents may be employed. In general, my process is applicable in those situations wherein a metal selected from the group consisting of iron, chromium, vanadium, nickel, cobalt, titanium and zirconium is formed by reacting a chloride of said metal with a reducing agent that is substantially more electropositive than said metal. Suitable reducing agents for the listed product metals are: magnesium, sodium, potassium, lithium, calcium, etc.

With few exceptions, the listed product metals are not utilized to any great extent in their pure form, being usually employed in the form of alloys in which said metal is the predominating metal present. My process is particularly suited to the production of these alloys. While there are a number of approaches to the production of an alloy in my process, it should always be the aim to cause each metal particle in the reaction product stream to conform in composition to the desired analysis. There being so many types of alloys of the listed base metals, it would be impossible to discuss the production of each alloy specifically; however, the basic approaches to alloy production will enable the user to produce any of the more common alloys presently being employed in industry.

If the alloying element is one having a chloride that is reducible by the reducing agent being employed to produce the base metal in the primary reaction zone, then the desired alloy may be produced by reacting said reducing agent with a mixture of chlorides in said primary reaction zone, the composition of the chloride mixture being such that its reduction yields particles of the desired alloy. If the alloying element is soluble in the reducing agent, such as is the case when aluminum is the alloying element and magnesium is the reducing agent, then the desired alloy is advantageously formed by feeding the aluminum required for the alloy formation into the primary reaction zone alloyed with the magnesium that is being fed into said zone. If desired, the alloying element may be fed directly into the pool of molten metal that forms the depositing surface of my process; however, it should be pointed out that this procedure will not yield a uniform composition as the foregoing procedures.

The formation of iron-carbon alloys offers an interesting problem in my process, however, as will be discussed later, the reduction of a mixture of ferric chloride and carbon tetrachloride, both in gas phase, will yield such alloys. In order to more clearly disclose the operation of my process, the following specific examples are given,

## Examples

In order to determine the efficiency of my process in forming an iron that was essentially free from carbon, hydrogen, sulphur and phosphorus, I chlorinated ordinary mild steel at an elevated temperature employing the general technique given by Lundell, Hoffman and Bright, Chemical Analysis of Iron and Steel, John Wiley & Sons, Inc., 1931, pages 413 thru 420, cylinder chlorine being freed from water for the purpose by freezing it out. The mild steel had the following composition:

|            | Percent |
|------------|---------|
| Carbon     | 0.14    |
| Manganese  | 0.42    |
| Silicon    | 0.09    |
| Phosphorus | 0.019   |
| Sulphur    | 0.027   |
| Copper     | 0.18    |
| Nitrogen   | 0.005   |

The test unit was a vertically-positioned pipe that was cooled by circulating water, much in the manner shown in Figure 2. The inside diameter of the pipe reactor was 2 and  $\frac{3}{4}$ ", the length being 24" from the top to the depositing surface. The length of the primary reaction zone was fixed at 10" by positioning the chlorine entrance ports 10" from the top of the reactor pipe, the chlorine entrance ports—2 in number—were formed of graphite pipe encased in stainless steel tubing, the steel tubing being water cooled in the area where they passed thru the water-jacket that formed the reactor wall. The unit was prepared for operation by removing the collecting (depositing) surface from the depositing chamber and preheating said surface to a red heat, the starting depositing surface being composed of rammed magnesia in the tests involving iron-base metals. The magnesia, consisting of pre-fused magnesia grains bonded with magnesium chloride, was rammed in the form of a plug that would slip easily up into the open bottom of the depositing chamber, much in the manner that shape 22 is positioned in Figure 3, however, during the tests, the depositing surface was positioned lower in the water-jacket mold 23 than shown in Figure 3, due to the fact that the tests were run on a batch basis; that is, the depositing surface was not lowered during the test runs in order to maintain the depositing surface at a fixed position within the mold, the deposited metal being allowed to build up until the top of the mold was reached or until the run was finished.

In the test runs involving the mild steel chlorides, I fed the mixed chlorides, in vapor phase, into the top of the reactor at the rate of about 125 grams per minute, at the same time that molten magnesium, at about 1050° K., was fed thereinto at a rate of about 60 grams per minute. This ratio of product metal chlorides to magnesium was more than a two-fold amount of magnesium over the stoichiometric proportion required to merely reduce the product metal chlorides to yield the product metals. After the primary reaction had been in operation for a short time, during which the water-jacket wall of the pipe reactor became coated with condensed magnesium chloride, I began the temperature build up phase of the process by feeding chlorine into the temperature build up zone at the rate of about 80 grams of chlorine per minute. This amount of chlorine was enough to oxidize a substantial portion, but not all, of the magnesium content of the reaction product stream. As soon as the chlorine introduction was commenced, the magnesia depositing surface was inserted in the depositing chamber in the path of the heated stream emerging from the temperature build up zone.

The byproduct chloride gas emerging from the depositing zone was exhausted from the depositing chamber thru an 8' length of 4" pipe. After a few minutes of operation, it became necessary to cool the exhaust pipe by means of a water spray, care being exerted so that the exhausting pipe was not cooled below the melting point of magnesium chloride, so as to avoid clogging the pipe.

This exhausting arrangement condensed a portion of the byproduct chloride gas, the balance being exhausted into the air where it formed a heavy smoke. The exhaust arrangement was effective in preventing air from diffusing into the reaction pipe, so that, once a few minutes operation had cleaned all hydrogen, oxygen and nitrogen out of the reactor, the entire reduction and collection process was carried out in the absence of these impurities.

After the depositing surface had been placed in position, the reduction/collection process was continued for 10 minutes; that is, as long as the supply of mixed chlorides held out. During this 10 minute interval, the input of iron was estimated at about 430 grams. The weight of the melted and solidified deposit collected on the depositing surface was 352 grams, reflecting a process yield of 81.8%. In spite of the absence of deoxidizers in the deposited iron, the small ingot took a shrink, indicating the absence of oxygen therein. Analysis of the top of the ingot showed:

|            | Percent          |
|------------|------------------|
| Carbon     | Less than 0.01.  |
| Manganese  | Trace.           |
| Silicon    | 0.03.            |
| Phosphorus | 0.005.           |
| Sulphur    | Less than 0.005. |
| Copper     | 0.02.            |
| Nitrogen   | Less than 0.001. |

The low nitrogen level at the top of the deposit demonstrated the ability of the process to clean up the reactor's atmosphere, for analysis of the first iron deposited showed 0.006% nitrogen.

A thermocouple positioned in the primary reaction zone showed a fairly uniform reading just over 1400° K throughout the 10 minute run.

While the manganese chloride and copper chloride content of the mixed chlorides were left behind when the iron chloride was distilled into the primary reaction zone, in other tests involving the reduction of the molten mixed chlorides with molten sodium, essentially all of the copper content and about 50% of the manganese content of the original mild steel were recovered in the deposited iron. In these tests employing sodium as the reducing agent, it was observed that sodium is not as efficient as magnesium in gaining the desired final temperature build up—this, in spite of the known higher activity of sodium. Thus, while 6 moles of magnesium would gain the desired temperature build up, 6 moles of sodium would not—3 moles being the equation requirement in both cases. With sodium, I was forced to employ 3 times the stoichiometric reaction proportion of the reducing agent in order to gain a deposit of the required type.

In another test run involving the use of my process for the production of a very low carbon stainless steel of the 18-8 type, I chlorinated an 18-8 to form a mixed chloride condensate. The composition of the 18-8 that was chlorinated:

|            | Percent |
|------------|---------|
| Carbon     | 0.07    |
| Manganese  | 0.55    |
| Silicon    | 0.44    |
| Phosphorus | 0.018   |
| Sulphur    | 0.021   |
| Chromium   | 18.48   |
| Nickel     | 8.75    |
| Nitrogen   | 0.07    |
| Zirconium  | 0.11    |

The melted mixed chloride condensate and molten magnesium were sprayed into the primary reaction chamber in substantially the same proportions as in the mild steel test run. The test was operated for 21 minutes during which the primary reaction zone functioned at about 1400° K. The 18-8 deposit recovered from this test reflected 68.9% of the calculated metal input. The top of the 18-8 deposit analyzed:

|            | Percent          |
|------------|------------------|
| Carbon     | Less than 0.01.  |
| Manganese  | 0.50.            |
| Silicon    | 0.27.            |
| Phosphorus | Trace.           |
| Sulphur    | Trace.           |
| Chromium   | 18.01.           |
| Nickel     | 8.70.            |
| Nitrogen   | Less than 0.001. |
| Zirconium  | None.            |

The failure of the silicon and zirconium to be efficiently recovered was due to their condition in the original 18-8, for another test demonstrated that these two elements could be efficiently recovered. In this latter test, I chlorinated a silicon-zirconium alloy of the following composition:

|           | Percent |
|-----------|---------|
| Silicon   | 50.11   |
| Zirconium | 37.78   |
| Iron      | 11.10   |
| Aluminum  | 0.92    |

In this test the proportions employed were about the same as in the previous tests, the reaction being instigated by distilling the mixed chlorides into a sprayed molten magnesium. Due to the separation that took place when the mixed chlorides were boiled off, the deposited metal was extremely segregated, the bottom of the deposit being essentially an alloy of iron and silicon, the top of the deposit being essentially pure zirconium, however, neither the top or the bottom of the deposit contained aluminum. Based upon the weight of the alloy consumed during the chlorination, the metal yield of the run was 70.5%.

In another test involving the production of titanium in my process, I chlorinated a ferro-titanium of the following composition:

|          | Percent |
|----------|---------|
| Carbon   | 0.05    |
| Titanium | 41.55   |
| Aluminum | 6.70    |
| Silicon  | 4.11    |
| Iron     | Balance |

By fractionally condensing the chloride gas, I separated most of the iron, the collected condensate containing mainly titanium and silicon tetrachlorides. The titanium and silicon chlorides were sprayed in the liquid form into a sprayed molten magnesium within the primary reaction zone in the following proportions: mixed chlorides, 100 grams per minute; molten magnesium, 50 grams per minute; chlorine, 65 grams per minute. These rates of feed were based upon the net feed during the run, 19 minutes, as were the feed rates in all of my tests, however, a certain measure of rate of feed variation occurred during the course of the run, due to variables which have no interest here. The yield of deposited metal during this 19 minute run was 72.8%, the composition of the melted deposit:

|          | Percent               |
|----------|-----------------------|
| Carbon   | Trace.                |
| Titanium | 88.9 (by difference). |
| Silicon  | 8.50.                 |
| Aluminum | Trace.                |

Feeling that the introduction of chlorine into contact with a metal product stream containing as active a metal as titanium would oxidize a substantial portion of the metal particle content of the reaction product stream, I arranged another test wherein I formed the test unit in the shape of a Y, the primary reaction zone occupying one arm, reaction in the other arm, so that the reaction product stream, formed with a moderate excess of magnesium, would merge with the heating stream at the point where the two arms met to form the base of the Y.

The process yield from this test was 78.5%, indicating that a certain amount of titanium oxidation did occur when chlorine was introduced directly into the temperature build up zone.

While the operating temperature of the primary reaction zone was in the vicinity of the boiling point of the reducing agent in most of my tests, in a few tests the temperature rose well over said boiling point, and it is noteworthy that the higher the temperature rose over this boiling point, the poorer the results, in terms of process yield. On the other hand, the mere fact that the primary reaction zone was operating at a temperature over the boiling point of the reducing agent should not be taken to mean that the reaction being entertained therein was a vapor phase reaction, for it was clear throughout my work that substantially all of the product metal yield arose from a reaction between the product metal chloride in gas phase and the reducing agent in liquid phase. The reasons why large product metal particles could be produced in a primary reaction zone operating at a temperature well above the boiling point of the reducing agent was due to the lag that occurred at the boiling point of the reducing agent, due to the latent heat of vaporization. In other words, as a given particle of molten reducing agent reacted with a gaseous environment containing the product metal chloride, the size of the mass of product metal being produced continued to increase until the entire system—reducing agent/metal product/reducing agent chloride—rose over the boiling point of the reducing agent, whereupon further reaction between the reactants in vapor phase yielded product metal particles too fine to be collected on the depositing surface. The higher the operating temperature, the quicker the system is lifted over this critical level, and the lower the process yield; however, it should be mentioned that acceptable yields can be obtained so long as the operating temperature is maintained below the boiling point of the reducing agent chloride.

As an indication of the sort of process yields obtainable when the operating temperature of the primary reaction zone is held at or over the boiling point of the reducing agent chloride, the following example may be given.

During the course of my work, it occurred to me that my preoccupation with a low operating temperature in the primary reaction zone might be unnecessary. Accordingly, I ran a strictly vapor phase test in a unit built somewhat in the manner of Figure 1. In this test, I fed molten magnesium and chlorine into the upper graphite chamber to form a highly heated stream consisting of magnesium chloride gas and magnesium gas, and then I flowed this highly heated stream into a primary reaction zone wherein ferric chloride gas was reacted with the magnesium gas content of the highly heated stream, the product stream from this reaction then being flowed into contact with the depositing surface. The yield from this test was 19.9%.

In another test of this vapor phase reaction, I reacted titanium tetrachloride with the highly heated stream containing magnesium and obtained a process yield of 16.2%. This test was of further interest due to the fact that the starting depositing surface was graphite instead of the usual magnesia. The bottom of the deposit ran 0.52% carbon, the top ran 0.17% carbon, and it was evident that this titanium deposit was ductile.

In view of the fact that the chlorination procedure employed to produce my product metal chlorides always eliminated substantially all of the carbon from the original metal, I experimented with the use of carbon tetrachloride for replacing this lost carbon, due to the importance of the carbon/iron, etc. alloys. I found that the introduction of carbon tetrachloride into the primary reaction zone resulted in the formation of the desired alloys containing carbon.

*The reactor*

While my invention does not involve reactor design, certain details of such design will be mentioned, so as to permit advantage to be taken of my experiences. As has been mentioned before, the primary reaction zone may be formed of a non-metallic refractory if the product metal will tolerate contact therewith. The use of a rammed lining of magnesia in a primary reaction zone wherein an iron alloy is being produced being an example of this. Other examples will occur to those skilled in the art. I prefer, however, to employ a water-jacket vessel to contain the primary reaction zone, the temperature build up zone and the depositing zone, such as is shown in Figures 2 and 3.

In Figure 1, the product metal depositing zone is shown containing a depositing surface consisting of a molten pool of product metal 8, the molten metal of pool 8 being caused to solidify at interface 9 by the cooling action of mold 12. As the product metal content of the heated stream collects on the depositing surface, the product metal shape that supports said surface is withdrawn in the indicated direction by conventional means (not shown) such as rolls. The product metal shape within mold 12 may be maintained in a controlled atmosphere by the introduction of fluid 10 in the indicated manner; that is, into the gap positioned between the solidified product metal shaped and mold 12, packing means 11 being positioned at the bottom of mold 12 in order to facilitate such atmosphere control. The reaction product streams are shown entering the heating stream. In passing thru the water-jacket and cooling water 7, said reaction product streams are naturally contained within suitable pipes (not shown).

Due to the cooling action of water 7 on the lining of the water-jacketed vessel, the reducing agent chloride deposits on said lining to form a heat-insulating layer that acts to minimize the heat losses in the process. There are a number of peculiarities concerning this deposit of reducing agent chloride. When a reactor first starts up, the reducing agent chloride deposits on the water-jacket to form a more or less porous frost, however, as the operation proceeds, this frost layer becomes more and more dense until, finally, it consists of a fused layer that is solid next to the bare water-jacket and molten next to the heated stream. The molten phase of this deposit is in the process of being continually formed and then flowing down the wall towards the molten depositing surface, and, unless the molten chloride is prevented from falling upon said molten surface, a continual series of explosions will occur in the reactor. While there are a number of methods for preventing this condensed, molten reducing agent chloride from falling on the depositing surface, I prefer to handle the situation as shown in Figures 1, 2 and 3. In Figures 1, 2 and 3, the depositing surface has the same shape and size as the cross section of the temperature build up zone in the same plane. In this connection, it is important that no dimension of said surface be larger than the corresponding dimension of the cross section of the temperature build up zone, and, while not shown in the figures, it is preferable that each dimension of said surface be smaller than the corresponding dimension of said zone. Under these design circumstances, the molten reducing agent chloride will flow into the by-product chloride gas chamber 14, either by entrainment in that portion of the heated stream that flows into chamber 14 without contacting the depositing surface, as shown by the flow lines in the figures, or by falling upon an inclined top 13 of the mold 12 containing the depositing surface, or both. The molten reducing agent chloride that flows into chamber 14 will quickly evaporate off, or it may be withdrawn in the molten state by means of an outlet (not shown). In the event that this molten chloride is removed from chamber 14 by evaporation, the product metal particles which it contains will remain behind in

chamber 14 to form accretions. Such accretions, and such other accretions of the product metal as may occur at undesired locations within the reactor, may be periodically removed by feeding chlorine or a reducible gas, such as ferric chloride, titanium tetrachloride, etc. in large excess into the atmosphere of the reactor for a short while. If desired, the product metal accretions within chamber 14 may be removed by feeding chlorine, ferric chloride, titanium tetrachloride, etc. into said chamber 14 by means of a suitable inlet (not shown) in said chamber 14. On the other hand, the development of such accretions within chamber 14 may be prevented by continuously feeding a substantial excess of such oxidizing gas into chamber 14, this procedure being compatible with the byproduct reducing agent chloride recovery and purification procedure previously disclosed.

The reactor of Figure 2 offers some design problems that differ from those of the reactor of Figure 1. In Figure 2, the heating stream is formed in a reaction chamber (not shown) that is separated from the reactor itself, the heating stream being flowed from the chamber in which it was formed into the temperature build up zone by means of suitable, refractory-lined pipes. The refractory lining of such pipes is preferably graphite, although other refractories will occur to those skilled in the art. Chlorine 28A is shown being introduced into the top of the reactor of Figure 2. This is an optional arrangement for gaining a preliminary temperature build up in the primary reaction zone or for periodically purging the reactor in order to remove accretions. Water-jacket 17 is shown forming the three contiguous phases of this synchronous process: the primary reaction zone, the temperature build up zone and the depositing zone, the depositing surface being formed by pool 42, pool 141 being supported by the iron shape that is formed at interface 15. The byproduct chloride gas 16 of Figure 2 is withdrawn from the vessel in the manners previously described. Inert gas 18 is shown being fed into the gap between the iron shape and the mold that formed said shape, packing 19 being employed to retain gas 18 within said gap.

Figure 3 pictures the use of chlorine in the temperature build up zone and the use of a separate, but contiguous, dichloride zone wherein the ferric chloride is first reduced to ferrous chloride, as previously described. The direct introduction of chlorine in the hot temperature build up zone requires certain precautions if attack on the vessel is to be avoided. In general, the chlorine must be led into said zone by means of cooled graphite pipes or other suitable refractory pipes. In Figure 3, depositing surface 20 is shown being supported by shape 22 that is formed from pool 48 at interface 21 within mold 23. The entire vessel, including that portion containing by-product chloride gas 24, is shown formed by a suitably designed water-jacket 51 containing cooling water 25.

*Miscellaneous factors*

While I have described the various embodiments of my process wherein the heat required in order to maintain the depositing surface at a temperature that lies above the boiling point of the reducing agent chloride being formed in the primary reaction zone is developed without the use of supplementary heating expedients, it seems plain that such supplementary heating may be employed, if desired. For example, the conduction of heat away from the depositing surface by flow downward along the product metal shape may be offset by inductively heating that portion of the product metal shape which extends below the mold. Other heating expedients will occur to those skilled in the art.

The Kelvin temperature scale is employed herein because it is the scale employed in Brewer's Tables: 3.7, 3.8, 6.3, 7.1 and 7.2, Chemistry and Metallurgy of Misc. Materials, McGraw-Hill Book Co., 1950, these tables being the best and most complete gathering together of data

concerning the melting points, boiling points, etc. of the metals, reducing agents and chlorides herein involved. In this connection, when I refer to the melting and boiling points of the various metals and chlorides herein involved, I naturally means the melting and boiling points exhibited by these metals, reducing agents and chlorides under the conditions which are characteristics of my process. One of these conditions is the relatively high pressure under which my process operates, due to the sudden and large expansion of the reducing agent chloride from a liquid to a gas within the confines of my process. Just how high this process pressure will be, in any given operation, will depend upon how the process is being operated and upon the back-pressure arising from the design of the outlet that withdraws the byproduct chloride gas from the reaction/collection vessel. This process pressure naturally has an elevating effect on the melting points and particularly the boiling points of the process reactants and resultants. Whatever the process pressure may be, however, when I refer to the boiling point of magnesium chloride, for example, I am referring to the boiling point exhibited by magnesium chloride under the environment obtained within my process vessel.

While I naturally prefer to operate my process in the absence of air and hydrogen, for the reasons previously given, the presence of these gases within my process is permissible if such is desired.

By definition, the reducing agents of my appended claims are those metals which are sufficiently electro-positive towards the subject product metal chloride to reduce said chloride with the formation of said metal; magnesium, calcium, sodium, potassium and lithium being examples of such reducing agent metals.

While I prefer to operate my heating process for the purposes hereinbefore stated, my heating process may be employed to merely heat treat the product metal particles contained in the subject reaction product. In other words, my temperature build up zone may be employed without the subsequent collection of the heated product metal particles in a consolidated form.

Having now described several forms of my invention, I wish it be understood that my invention is not to be limited to the specific arrangements hereinbefore described and shown, except insofar as such limitations are specified in my appended claims.

I claim as my invention:

1. In the process wherein a chloride of an element selected from the group consisting of iron, chromium, vanadium, nickel, cobalt, titanium and zirconium is reacted in a reaction zone with a reducing agent metal selected from the group consisting of magnesium, calcium, sodium, potassium and lithium to form a reaction product containing a product metal in which at least one of said elements is a major constituent and a chloride of said reducing agent metal, and in which said product metal is then separated from said reaction product, the method of separating said product metal from said reaction product, which comprises: flowing said reaction product to form a reaction product stream in which particles of said product metal are dispersed within a molten stream of said reducing agent metal chloride, the temperature of said reaction product stream being in the range between above the melting point and below the boiling point of said reducing agent metal chloride; flowing said reaction product stream into a temperature build-up zone that is essentially separate from said reaction zone; reacting sufficient chlorine gas with sufficient of said reducing agent metal in fluid phase to form a heating stream of a gas consisting essentially of a chloride of said reducing agent metal at a temperature that lies substantially above the boiling point of said reducing agent metal chloride; mixing said reaction product stream with sufficient of said heating stream within said temperature build-up zone to

- lift the resulting mixed stream to a temperature that lies above the boiling point of said reducing agent metal chloride; flowing said mixed stream into a contiguous depositing zone wherein particles of the product metal content of said mixed stream are brought into contact with and collected on the heated surface of a mass of said product metal by flowing said mixed stream into contact with said surface, said surface being maintained at a temperature that lies above the boiling point of said reducing agent metal chloride with the aid of the heat content of said mixed stream; and then flowing the gas content of said mixed stream away from said surface.
2. The method according to claim 1 in which said reaction product stream contains said reducing agent metal and in which the temperature of said reaction product stream is lifted by reacting the reducing agent metal content of said reaction product stream with chlorine gas within said temperature build-up zone.
3. The method according to claim 2 in which said reaction between the reducing agent metal content of said reaction product stream and chlorine gas lifts said reaction product stream above the boiling point of said reducing agent metal chloride.
4. The method according to claim 1 in which said heating stream is formed by reacting said reducing agent metal with a stoichiometric excess of chlorine gas.
5. The method according to claim 1 in which said heating stream is formed by reacting chlorine gas with a stoichiometric excess of said reducing agent metal.
6. The method according to claim 1 in which said reaction product stream is formed in said reaction zone and is then flowed downward into a contiguous temperature build-up zone wherein sufficient of said heating stream is mixed with said reaction product stream to lift the resulting mixed stream to a temperature that lies above the boiling point of said reducing agent metal chloride; in which said mixed stream is then flowed downward into a contiguous depositing zone wherein said mixed stream is flowed into contact with said heated surface to collect a substantial portion of the product metal content of said mixed stream on said heated surface; and in which the gas content of said mixed stream is then flowed away from said heated surface.
7. The method according to claim 6 in which said reaction zone is divided into two contiguous reaction zones, the first of which being employed to conduct a reaction between said reducing agent metal and a stoichiometric excess of said chloride of said element, said chloride being oxidizing towards said element, to form a first reaction zone reaction product stream consisting of said reducing agent metal chloride, a lower chloride of said element and said excess of said oxidizing chloride; and in which the reaction product stream from said first reaction zone is then flowed downward into a contiguous second reaction zone wherein said first reaction zone reaction product stream is reacted with a stoichiometric excess of said reducing agent metal to form a second reaction zone reaction product stream containing particles of said product metal dispersed in a molten stream of said reducing agent metal chloride, said second reaction zone reaction product stream being then flowed downward into said contiguous temperature build-up zone.
8. The method according to claim 1 in which said heated surface is maintained at a temperature in the range between above the boiling point of said reducing agent metal chloride and below the melting point of said product metal.
9. The method according to claim 1 in which said heated surface is maintained at a temperature that lies above the melting point of said product metal.
10. The method according to claim 1 in which said product metal consists of an alloy of said element with at least one other element and in which said alloy is pro-

duced in said reaction zone by reacting a mixture of chlorides with said reducing agent metal.

11. The method according to claim 1 in which said heated surface is the surface of a pool of a molten alloy consisting of said element and at least one other element and in which said other element is introduced into said pool by feeding said other element into said pool.

12. The method according to claim 1 in which sufficient chlorine gas is introduced into the gas stream after it has flowed away from said heated surface to oxidize product metal particles entrained in said byproduct chloride gas stream to the highest state of oxidation obtain-

able at the temperature involved, and in which the resulting stream is then fractionally condensed to separate the components thereof.

References Cited in the file of this patent

UNITED STATES PATENTS

2,205,854 Kroll ----- June 25, 1940  
2,668,750 Krchma ----- Feb. 9, 1954

FOREIGN PATENTS

505,801 Belgium ----- Sept. 29, 1951